

# UNITED STATES PATENT OFFICE.

SEIICHI SAKANE, OF KAMIKYO-KU, JAPAN.

## PROCESS OF EXPANDING THE CROSS SECTIONS OF SPUN-SILK YARN.

1,413,193.

Specification of Letters Patent. Patented Apr. 18, 1922.

No Drawing.

Application filed December 8, 1920. Serial No. 429,153.

To all whom it may concern:

Be it known that I, SEIICHI SAKANE, a subject of the Emperor of Japan, residing at No. 370 Motoshinnyodo-cho, Kamikyo-ku, Kyoto, Japan, have invented new and useful Improvements in a Process of Expanding the Cross Sections of Spun-Silk Yarn, of which the following is a specification.

This invention relates to a process of expanding the cross section of a spun-silk yarn by counter twisting the said yarn and steaming it. It has for its object to make elastic and soft woolly yarn of spun-silk. The expression "spun-silk" is used here in a broad sense; it is used to mean not only ordinary silk that is spun but those of mandarin silks, Japanese oak silks, Chinese oak silks and the like. Silk yarn containing cotton or woollen portions may also be profitably treated by this new process.

To describe further, to treat twisted single yarn, it is at first heated in dry or wet state for twenty or thirty minutes, so that the curling of silk fibres in the said yarn may be made permanent. Where the yarn has been already heated in a previous treatment, such for instance as bleaching, scouring or dyeing so that the curling of the silk fibres has become permanent, the preparatory treatment above described may be dispensed with.

The yarn thus treated after being dried, is then counter twisted, by any suitable twisting machine in order to untwist about a half or one third of the total number of twists of the yarn. After untwisting, the silk fibres of the yarn become separated one from the other, thereby expanding the cross section of the yarn.

Next the yarn is reeled on a swift and made into a hank by any suitable means such, for instance, as by winding it loosely on a pair of parallel bars. The hank is then steamed so as to prevent the yarn from re-twisting but is left free to shrink. In about five minutes of steaming, the silk fibres are permanently set in their separated condition and, consequently, the cross section of the treated yarn gets larger and the yarn becomes elastic, soft and woolly. It looks like woollen yarn but is more lustrous.

Doubled yarn may be treated in the same way. When it is steamed and counter twisted, the single yarns of which the twine is

made and the silk fibres in the single yarns respectively separate themselves from one other, thereby expanding the cross section of the doubled yarn. The single yarns and their fibres are permanently set in separated condition in a succeeding steam-treatment.

Instead of the preparatory steaming and untwisting in the process of above mentioned, another method may be used for doubled yarn. Single yarns, of which doubled yarn is to be made, are first twisted in a required number of filatures, and then they are twined by a doubling machine so as to produce a number of twists corresponding to about half the number of the filatures. For example, when two single yarns of spun-silk 70 yarn of 120 ply are to be doubled, the number of twists or filatures of the single yarns is 472 per meter in the metric system, while the corresponding number of twists is 425 per meter. In the present method, the number of twists is reduced to about from 200 to 300 per meter, so that the tendency of the single yarns to further twist is the same as when a twisted yarn is untwisted by the method first described. The succeeding 80 treatment, that is to say, steaming should be done next. The same result may be attained by this modified method as by means of that first mentioned.

I claim:

1. The process of expanding the cross section of spun-silk yarn which consists in counter twisting the twisted yarn, and subjecting the yarn to steam-treatment while keeping said yarn free to shrink but preventing it from twisting back.

2. The process of expanding the cross section of spun-silk yarn which consists in counter twisting about half of the total number of twists of the twisted yarn, and subjecting the yarn to steam-treatment while keeping said yarn free to shrink but preventing it from twisting back.

3. The process of expanding the cross section of twisted yarn which consists in twisting single yarns, doubling said yarns so as to produce a number of twists corresponding to approximately half the total number of twists or filatures of the single yarns, and subjecting the yarn to steam-treatment, while keeping the yarn free to shrink but preventing it from twisting.

SEIICHI SAKANE.